

Jan. 2, 1945.

H. A. DIEHL ET AL

2,366,185

ROLLING COMPOSITE MAGNESIUM-BASE ALLOY SHEETS

Filed May 4, 1942



*Fig. 1*



*Fig. 2*

INVENTORS  
Harold A. Diehl  
John C. McDonald  
BY

Griswold & Burdick  
ATTORNEYS

## UNITED STATES PATENT OFFICE

2,366,185

## ROLLING COMPOSITE MAGNESIUM-BASE ALLOY SHEETS

Harold A. Diehl, Bay City, and John C. McDonald,  
Midland, Mich., assignors to The Dow Chemical  
Company, Midland, Mich., a corporation of  
Michigan

Application May 4, 1942, Serial No. 441,728

3 Claims.

(Cl. 29—189)

This invention relates to an improved method of bonding together sheets formed of magnesium or plastically deformable magnesium-base alloys.

Composite articles consisting of sheets of two or more different magnesium-base alloys united by a firm bond are desirable for a variety of structural purposes. In particular, sheets consisting of a core metal formed of an alloy characterized by extreme strength clad with a thin layer of an alloy of the highly corrosion resistant type are especially useful in that such composite sheets exhibit a combination of the desirable properties of both alloys without the disadvantages of either. A number of methods for forming such composite sheets are known, but none provides a bond between the two sheets which is strong enough to withstand without rupture the severe stresses to which the sheets sometimes are subjected during fabrication and use.

An object of the present invention, then, is to provide an improved method of making composite articles formed of magnesium and a magnesium-base alloy or of two or more different magnesium-base alloys in which the individual sheets forming the article are held together by a firm strong bond capable of resisting all stresses to which such articles are ordinarily subjected.

The accompanying drawing shows in Fig. 1 a cross-section of a pair of magnesium-base alloy sheets tack welded at the edges, and Fig. 2 is a similar view of the same sheets on being pressed between a pair of rolls of a rolling mill.

Bonding of magnesium-base alloy sheets according to the invention is accomplished by rolling together the sheets at a temperature between 750° and 900° F. and at a rate of reduction in thickness of at least 40 per cent per pass through the rolls. The generation of heat and the mechanical working accompanying the rolling appear to cause an interaction, possibly a diffusion of metal, between the two adjacent surfaces, and thus to form a firm strong bond between the sheets.

In practice, the magnesium or magnesium-base alloy sheets are first carefully cleaned to remove mill scale, organic matter, and any chemical finish which may be present, preferably by sanding. The clean sheets to be bonded are then laid one upon another and are gripped together firmly by mechanical means, as by passing wire or steel tape around the sheet and drawing it tight, or by "tacking" the sheets together at the edges by welding as shown in Fig. 1. The resulting stack of two or more sheets is then transferred to a

suitable oven and heated to a temperature in the range 750° to 900° F., preferably above 800° F.

The hot pack of sheets is then removed from the oven and passed once or preferably several times through a conventional rolling mill adjusted to produce a reduction in thickness of the pack per pass of at least 40 per cent, reductions in the range 40 per cent to 75 per cent per pass being preferred as shown in Fig. 2. After the rolling step, the wires or other securing means may be removed from the pack. The original sheets constituting the pack are found to be bonded together firmly. The composite article thus formed may then be subjected to further rolling and annealing operations as desired to develop any range of physical characteristics of which the metal is capable, and may be cut, punched, drawn, or otherwise shaped without danger of rupturing the bond between the original sheets.

In so far as is known, the process of the invention may satisfactorily be applied to bonding magnesium or any plastically deformable magnesium-base alloy to any other plastically deformable magnesium-base alloy. As a practical matter, however, the invention finds its greatest application in bonding high strength magnesium-base alloys containing aluminum in a proportion up to 10 per cent as the major alloying element to highly corrosion resistant magnesium-base alloys containing manganese in a proportion up to 2 per cent as the major alloying element. In this way there is formed a composite article having a high strength core and surfaces of high corrosion resistance.

The following example will illustrate the invention but is not to be construed as limiting its scope:

## Example

40. A 0.47 x 8 x 8 inch extruded slab of Dowmetal FS (a magnesium-base alloy containing 2.7 per cent aluminum, 0.3 per cent manganese, and 1.0 per cent zinc, the balance being substantially magnesium) and two 0.040 inch thick sheets of 45. annealed Dowmetal M (a magnesium-base alloy containing 1.5 per cent manganese, the balance being substantially magnesium) were carefully cleaned by sanding. The cleaned sheets were then superimposed with the thick sheet in the middle and were secured together by welding along the edges. The resulting pack was then placed in a furnace and heated to a temperature of 900° F., after which the heated pack was passed repeatedly between rolls at a rate of reduction in thickness per pass of 50 per cent with 50. 55.

reheating to temperature between passes until a final thickness of 0.075 inch was reached. The composite sheet thus produced exhibited a firm tight bond between the individual sheets of which it was formed.

Other modes of applying the principle of the invention may be employed instead of those explained, change being made as regards the details described, provided the steps recited in any of the following claims or the equivalent thereof are used.

We claim:

1. The method of bonding together sheets formed of magnesium or plastically deformable magnesium-base alloys which comprises rolling the unbonded sheets together at a temperature between 750° and 900° F. at the rate of reduction in thickness of at least 40 per cent per pass through the rolls.
2. The method of bonding together sheets formed of different plastically deformable mag-

nesium-base alloys which comprises superimposing the sheets to be bonded, heating them to a temperature in the range 750° to 900° F., and passing the heated unbonded sheets together through rolls at a rate of reduction in thickness per pass of at least 40 per cent.

3. The method of bonding a sheet formed of a plastically deformable magnesium-base alloy containing aluminum in a proportion up to 10 per cent as the major alloying element to a sheet formed of a magnesium-base alloy containing manganese in a proportion up to 2 per cent as the major alloying element, which comprises superimposing the sheets to be bonded, heating them to a temperature in the range 750° to 900° F., and passing the heated unbonded sheets together through rolls at a rate of reduction in thickness per pass of 40 per cent to 75 per cent.

HAROLD A. DIEHL.  
JOHN C. McDONALD.